# EUROPEAN PATENT SPECIFICATION

(11) **EP 0 477 383 B1**
(45) Date of publication and mention of the grant of the patent: **07.02.1996**
(21) Application number: 91906694.4
(22) Date of filing: 08.04.1991
(51) Int. Cl.: C22C 9/00, C22C 38/20, C22C 38/28, C22C 38/32, C22C 38/36

(54) **IRON-COPPER ALLOY PLATE WITH ALLOY STRUCTURE EXCELLENT IN HOMOGENEITY**
EISEN-KUPFER-BAND MIT AUSGEZEICHNET HOMOGENER GEFÜGESTRUKTUR
TOLE EN ALLIAGE DE FER ET DE CUIVRE AVEC STRUCTURE ALLIEE A EXCELLENTE HOMOGENEITE

(30) Priority: 09.04.1990 JP 93440/90
(43) Date of publication of application: 01.04.1992
(73) Proprietor: NIPPON STEEL CORPORATION, Tokyo 100-71 (JP)
(72) Inventor: UESHIMA, Yoshiyuki, Kimitsu Seitetsusho, Kimitsu-shi, Chiba 299-11 (JP); MIZOGUCHI, Toshiaki, Kimitsu Seitetsusho, Kimitsu-shi, Chiba 299-11 (JP); MIYAZAWA, Kenichi, Kimitsu Seitetsusho, Kimitsu-shi, Chiba 299-11 (JP); NISHIMURA, Satoshi, Daini Gijutsu Kenkyusho, Sagamihara-shi, Kanagawa 229 (JP)
(74) Representative: Carter, Caroline Ann
(86) International application number: JP9100463
(87) International publication number: WO9115608

(56) References cited:
- JP-A- 6 270 541
- JP-A-63 149 344
- No further relevant documents have been disclosed.

## Description

The present invention relates to an Fe-Cu alloy sheet having an alloy structure of high uniformity which can be used as a material for electronic and magnetic parts or the like. The invention also relates to alloys suitable for use in making the sheets.

Conventionally, Kovar (Fe-29Ni-16Co), 42 Alloy (Fe-42%Ni), stainless steel disclosed in JP-A-63-293143 and so on have been used as a material for electronic and magnetic parts in semiconductor equipment or the like. However, those alloys have a problem that they are expensive, and they also have a problem that they are inferior in conductivity and heat-radiation efficiency. In order to improve these characteristics, therefore, a copper (Cu) base alloy has come into use recently.

The Cu-base alloy of which copper content is 90% or more is low in the strength. Consequently, iron is added to the Cu-base alloy as a strengthening element, and chromium is added to it, as disclosed in JP-A-49-91025 (an alloy for sliding contact parts of electric equipment) or the like, so as to improve the corrosion resistance property as well. Moreover, as disclosed in Iron and Steel Handbook, the third edition, Vol. IV, pp. 211 - 212 (compiled by Japan Iron and Steel Association), adding molybdenum to improve the corrosion resistance property is a known method. The problem is, however, that additions of such alloying elements cause the uniformity of the alloy to deteriorate.

It should be noted that the Fe-Cu-Cr alloy which is disclosed in JP-A-49-91025 is not intended as a material for electronic and magnetic parts. Although the stainless steel for an electronic material which is disclosed in JP-A-63-293143 is intended for the same kind of use, it has obviously different elements in the compositions. Further, an alloy strip manufacturing method disclosed in JP-A-60-152640 is obscure in the kind of composition, restriction of additive elements, and effective concentration ratios. Furthermore, none of these preceding techniques discloses any suggestion concerning the manufacture of an Fe-Cu alloy having high uniformity which is the object of the present invention, so that it is doubtful whether such an alloy can be manufactured or not.

Among Fe-Cu alloys, for example, an alloy containing 50% copper exhibits a uniform liquid phase unless it contains chromium. However, if it contains 3% or more chromium, when it is melted, it becomes a molten liquid which separates into a liquid phase rich in iron and another liquid phase rich in copper. If such an alloy having two separate phases, i.e., the liquid phases rich in iron and copper respectively, is cast, a uniform product cannot be obtained. That is to say, regions of the iron-rich liquid phase and regions of the copper-rich liquid phase increase in size during the melting operation, and, after they solidify, cracks are generated in interfaces between those two phases during cold working, causing disadvantages such as poor bending characteristics of final products.

Thus, it is an object of the present invention to produce an alloy sheet having a fine and uniform structure according to a thin plate continuous casting method. In accordance with the invention, particular elements are included in an Fe-Cu-Cr alloy or an Fe-Cu-Cr-Mo alloy so as to solve the problem of non-uniformity of the alloy structure due to the above-described phenomenon that regions in the liquid phase rich in iron and regions in the liquid phase rich in copper increase in size during the melting operation.

With respect to the above-mentioned object of the invention, there are provided alloy sheets as follows:
(1) An Fe-Cu alloy sheet manufactured by a thin plate continuous casting method, the alloy containing, by weight, 20 to 90% Cu, 1 to 10% Cr, 0 to 10% Mo, and one or more alloying elements selected from the group consisting of Aℓ, Sc, Y, La, Si, Ti, Zr and Hf whose amount or total amounts are not less than a calculation value of the following expression and not more than 10%, the balance, apart from impurities, being Fe: wherein α = 1,
   β = 51 - [% Cu] (in the case where Cu = 20 to 50%),
   β = -19 + 0.4 [% Cu] (in the case where Cu = 50 to 90%) and
   further, | [% Cu] - 50 | is an absolute value of "% Cu - 50".
(2) An Fe-Cu alloy sheet manufactured by a thin plate continuous casting method, the alloy containing, by weight, 20 to 90% Cu, 1 to 10% Cr, 0 to 10% Mo, and boron (B) and/or carbon (C) whose amount or total amounts have a lower limit value which is a calculation value of the following expression, and have an upper limit value which is 1% when only boron is present and when boron and carbon are present, and which is 3% when only carbon is present, the balance, apart from impurities, being Fe: wherein α = 0.01,
   β = 51 - [% Cu] (in the case where Cu = 20 to 50%),
   β = -19 + 0.4 [% Cu] (in the case where Cu = 50 to 90%).
(3) An Fe-Cu alloy sheet manufactured by a thin plate continuous casting method, the alloy containing, by weight:
   20 to 90% Cu;
   1 to 10% Cr;
   0 to 10% Mo;
      one or more alloying elements selected from the group consisting of Aℓ, Sc, Y, La, Si, Ti, Zr and Hf whose amount or total amounts are not less than a calculation value of the following expression and not more than 10%; and
      boron and/or carbon whose amount or total amounts have a lower limit value which is a calculation value of the following expression, and have an upper limit value which is 1% when only boron is present and when both boron and carbon are present, and which is 3% when only carbon is present, the balance, apart from impurities, being Fe:
   the expression being wherein α = (in the case where the amounts of elements belonging to the group comprising Aℓ, Sc, Y, La, Si, Ti, Zr and Hf are calculated),
   α = 0.01 (in the case where the amounts of B and/or C are calculated),
   β = 51 - [% Cu] (in the case where Cu = 20 to 50%),
   β = -19 + 0.4 [% Cu] (in the case where Cu = 50 to 90%).

The invention also provides alloys suitable for use in making the sheets of the invention, the alloys having the compositions specified in (1), (2) and (3) above. The alloy sheets of (1), (2) and (3) above have alloy structures of high uniformity.

The invention further provides the use of one or more alloying elements, in an Fe-Cu alloy, the nature and amount of the alloying elements used and the composition of the Fe-Cu alloy being as described in (1), (2) and (3) above, to reduce separation of molten forms of the alloy into iron-rich and copper rich phases.

The alloy plate according to the present invention may be used as a material for electronic and magnetic parts, and is made of the alloy whose basic alloy components are iron and copper, the alloy containing copper in a range of 20% to 90%. The alloy contains at least 20% or more copper in order to enhance the electric conductivity. Iron is also included in the alloy for improving the strength of the alloy. The range of iron content varies in accordance with the purpose for which the alloy is to be used, and it is balanced with the electric conductivity and the strength and determined in relation with other additive elements. However, if iron is added excessively, the corrosion resistance may deteriorate. Chromium is included in a range of 1 to 10% so as to improve corrosion resistance. However, since chromium increases repulsive forces between the atoms which are the alloy components in the molten metal, there is induced separation into two phases, i.e., the liquid phase rich in iron and the liquid phase rich in copper. Although molybdenum is added as occasion demands, it may cause the same kind of phenomenon as in the case of chromium. As described previously, if the molten metal having two separate phases is cast as it is, coarse crystalline grains of the phase rich in iron and the phase rich in copper will exist in castings. Therefore, it is difficult to work such metal into a material for electronic equipment and the like, and there are induced disadvantages in relation to characteristics of final products.

In one aspect of the present invention, one or more alloying elements selected from the group consisting of Aℓ, Sc, Y (yttrium), La, Si, Ti, Zr and Hf are added to the above-mentioned basic components, and this addition has the effect of suppressing the separation into two coarse phases of the above-described base alloy. In other words, when these alloying elements are added to the molten metal, attraction forces between the elements are enhanced when they are melted so that the liquid phase will not separate into two phases. It is necessary to add one or more alloying elements selected from the group described above, the amounts of which are not less than a calculation value of the following expression: wherein α = 1,
β = 51 - [% Cu] (in the case where Cu = 20 to 50%),
β = -19 + 0.4 [% Cu] (in the case where Cu = 50 to 90%).

If the above expression has a negative value, the lower limit value of the content is set to be zero. As a result of experimentation by the inventors, the above equation was obtained, in the case where the alloy contains at least one element selected from the group consisting of Aℓ, Sc, Y, La, Si, Ti, Zr and Hf (hereinafter referred to as X₁ element(s)), by determining quantitatively the relationship between the proportions of chromium and molybdenum, which promote the separation into two phases, and the lower limit value of the amount of X₁ element(s). If X₁ element(s) is or are added excessively, it/they will dissolve in the phase rich in copper, thereby causing the electric conductivity to deteriorate. Consequently, the amount of X₁ element(s) must not exceed 10%.

Another aspect of the invention is based on the fact that boron (B) and carbon (C) have substantially the same effect as the above-described group of X₁ element(s). Thus, at least one of those elements (hereinafter referred to as X₂ element(s)) may be added, the lower limit value of which is a value obtained from the above expression with α = 0.01. However, if X₂ element(s) is or are added excessively, coarse precipitates (for example, Fe₂B, Fe₃C) are generated, thus embrittling the structure. Therefore, the content should not exceed 1% when only boron is added or when boron and carbon are both included in the alloy, and should not exceed 3% when only carbon is used. Either one or more elements from the X₁ element group or one or more elements from the X₂ element group may be used, or alternatively, at least one element from each of the groups may be used together.

Other characteristics of the present invention will be obvious from the description below with reference to tables and the attached drawings.

In the drawings:
Fig. 1 is a schematic view of a twin-roll continuous casting apparatus for use in making an alloy sheet in accordance with the invention; and
Figs. 2a and 2b are graphs exhibiting relationships between amounts of additive components of the invention and the structure fineness.

In accordance with the present invention, Fe-Cu alloy sheets containing the above-described elements are manufactured by a thin plate continuous casting method. Especially, a thin casting with a thickness of 10 mm or less is produced. In this casting method, twin rolls are preferably employed. More specifically, as schematically shown in Fig. 1, cooling twin rolls 1 and 2 are provided with a pressing device 3 for castings. Molten metal from a molten metal pool 4 formed by the rolls 1, 2 and a side dam 5 is cooled by the twin rolls 1, 2 and turned into solidified shells 6, which are pressed by the pressing device 3 and drawn as a thin casting 7. The casting thus produced has an extremely fine and uniform structure because the casting, which can be formed as a thin plate of 5 mm or less, is cooled rapidly and contains the X₁ and/or X₂ element(s) mentioned above. Needless to say, however, the invention is not limited to the twin-roll casting method, and other methods (for example, a single-roll method, a belt casting method, and a caterpillar type casting method) may be employed so long as a thin-plate casting having a thickness of 10 mm or less can be obtained.

The above-described thin casting can be cold-rolled without hot-rolling so as to obtain a final product with a desired thickness or an intermediate material. If the alloy of the invention is hot-rolled, the alloy will become brittle when it is heated, for instance, to a temperature of 1000°C or more, so that hot-rolling of the alloy may become difficult. In the present invention, therefore, the casting is intended to have a thickness of 10 mm or less in order that it can be cold-rolled directly. Besides, in the twin-roll method, there can be obtained castings having a thickness of 5 mm or less, as described previously, and it is advantageous to carry out a cold rolling operation. After the cold-rolling operation, the castings are subjected to annealing treatment and the like, or if necessary, they are plated or punched. Thus, they can be turned into desired products, for example, electromagnetic materials and sheet products such as lead frames, and various forms of wire and foil.

### EXAMPLE 1:

Various kinds of the X₁ and/or X₂ element(s) in different amounts were added to the basic alloy materials (Fe-Cu system alloys) 1 to 3 shown in Table 1 and to two further alloys, 4 and 5, identified below Table 1. After a mixture of the X₁ and/or X₂ element(s) and one of the basic alloy materials in total amounts of 1 kg was melted in a magnesia crucible at 1510°C, the melt was brought into contact with a chilled member of copper and thereby cooled down rapidly. Thus, a plurality of samples were obtained. Cross-sections of the rapidly cooled samples (4 mm thick) thus obtained were observed by use of an optical microscope, and the structure fineness of each sample was examined to investigate the structure uniformity.

Tables 2 to 6 show values of the structure fineness for every X₁ and/or X₂ element corresponding to content ratios defined by the following equation: It should be noted that the structure fineness in this case means a maximum grain size.

Two further Fe-Cu basic alloys (alloys 4 and 5) were used, each containing Cu, Cr and 0.05% Mo.

Concerning any of the above-described basic alloy materials (samples), when each of the X₁ and X₂ elements of amounts corresponding to the content ratio of 1 were added, the structure became drastically finer and had no coarse structure of the two phases (the phase rich in iron and the phase rich in copper).

### EXAMPLE 2:

Referring to Table 7, 50%Cu-6%Cr-Fe alloys to which each of Aℓ and Ti was added at six levels in a range of 0.1 to 5% were melted, and castings were manufactured from them by a twin-roll method which will be shown in Fig. 1. Rolls made of a copper alloy having a diameter of 30 mm and a width of 10 mm were used as cooling twin rolls 1, 2 in a continuous casting apparatus according to this twin-roll method. The casting operation was conducted under such conditions as a casting temperature of 1510°C and a roll rotating speed of 20 rpm, and castings having a thickness of 2.2 mm were obtained. Cross-sections of the castings were observed by use of an optical microscope, and structure fineness of each casting was measured. Results of the measurement are shown in Figs. 2a and 2b (reference symbol □ indicates a sample containing aluminum and reference symbol indicates a sample containing titanium).

As may be clearly understoodfrom Figs. 2a and 2b, when the X₁ element(s) having amounts corresponding to the content ratio of less than 1 were added, they had the coarse structure divided into the two phases, and when the x₁ element(s) having amounts corresponding to the content ratio of 1 or more were added, the structure became drastically finer.

Examination results of the X₁ component(s) of the example 1 (indicated by slant-line portions) are also shown in Figs. 2a and 2b. It is obvious from Fig. 2a that the basic alloy materials 1 to 3 of the example 1 exhibited substantially the same tendency as the example 2. As for the basic alloy materials 4 and 5 of the example 1, however, shifts in a direction of the axis of abscissas were observed, and consequently, a correction factor β was introduced into the denominator of the equation defining the content ratio which is the index of the abscissas, so that the examination results would be uniform, as shown in Fig. 2b.

Table 7 shows results of evaluations in working characteristics (examinations of cracks in cold-rolled sheets) and physical properties for lead frame materials (critical numbers of cyclic bending in rupture tests and the corrosion resistance property) of the alloys thus obtained. More specifically, the above-mentioned castings designated by sample numbers 1 to 12 which had a thickness of 2.2 mm were first subjected to softening annealing treatment at a temperature of 800°C for one hour. After that, they were immersed, at a speed of 1 m/min., in a tank of 1.5 m which contained 10-volume% nitric acid solution heated at a temperature of 50°C so as to subject the iron phase to selective etching treatment. After that, the primary cold-rolling of these samples was performed at a reduction of 85%, and the examinations of cracking in cold-rolled sheets were conducted. Next, the samples which had undergone the crack examinations were annealed at a temperature of 550°C for three hours. In the course of the succeeding cooling process, they were aged at a temperature of 480°C for three hours. After that, they were cooled down to a temperature of 100°C at a rate of 50°C/hour, and the secondary cold-rolling of them was performed at a reduction of 8% to thereby obtain sheets having a thickness of 0.3 mm as the final products.

Bending tests of the product sheets thus obtained were conducted in the following manner so as to determine the critical numbers of cyclic bending operations in rupture tests. More specifically, the center of each product sheet having a width of 10 mm and a length of 50 mm was clamped by a vice and repeatedly bent at an angle of 90° along a circular arc having a radius of 0.25 mm. The number of bending operations until the product sheet was ruptured was counted and recorded as the critical number of cyclic bending operations in the rupture test.

As to the corrosion resistance property, the samples whose red rust generation rate exceeded a criterion of Fe-42Ni level as a result of a salt spray test for 48 hours were judged to be approved.

It can be understood from Table 7 that the materials containing aluminum or titanium whose content was 1% or more exhibited favorable results in the examination of cracks in cold-rolled sheets, the critical number of bending operations in rupture test and the corrosion resistance (the samples of the invention), and that the samples 1 to 3 and 7 to 9 having less than 1% aluminum or titanium were all rejected.

According to the present invention, there can be obtained alloy materials which have excellent cold working characteristics and excellent physical properties, and which have an extremely fine structure without separating into two phases when they are melted, so that they will be suitably used as materials of electronic and magnetic parts or the like.

## Claims

1. An Fe-Cu alloy sheet manufactured by a thin plate continuous casting method, the alloy containing, by weight, 20 to 90% Cu, 1 to 10% Cr, 0 to 10% Mo, and one or more alloying elements selected from the group consisting of Aℓ, Sc, Y, La, Si, Ti, Zr and Hf whose amount or total amounts are not less than a calculation value of the following expression and not more than 10%, the balance, apart from impurities, being Fe: wherein α = 1,
β = 51 - [% Cu] (in the case where Cu = 20 to 50%),
β = -19 + 0.4 [% Cu] (in the case where Cu = 50 to 90%).

2. An Fe-Cu alloy sheet manufactured by a thin plate continuous casting method, the alloy containing, by weight, 20 to 90% Cu, 1 to 10% Cr, 0 to 10% Mo, and boron and/or carbon whose amount or total amounts have a lower limit value which is a calculation value of the following expression, and have an upper limit value which is 1% when only boron is present and when both boron and carbon are present and which is 3% when only carbon is present, the balance, apart from impurities, being Fe: wherein α = 0.01,
β = 51 - [% Cu] (in the case where Cu = 20 to 50%),
β = -19 + 0.4 [% Cu] (in the case where Cu = 50 to 90%).

3. An Fe-Cu alloy sheet manufactured by a thin plate continuous casting method, the alloy containing, by weight:
20 to 90% Cu;
1 to 10% Cr;
0 to 10% Mo;
one or more alloying elements selected from the group consisting of Aℓ, Sc, Y, La, Si, Ti, Zr and Hf whose amount or total amounts are not less than a calculation value of the following expression and not more than 10%; and
boron and/or carbon whose amount or total amounts have a lower limit value which is a calculation value of the following expression, and have an upper limit value which is 1% when only boron is present and when both boron and carbon are present and which is 3% when only carbon is present, the balance, apart from impurities, being Fe:
wherein α = 1 (in the case where the amounts of elements belonging to the group consisting of Al, Sc, Y, La, Si, Ti, Zr and Hf are calculated),
α = 0.01 (in the case where the amounts of boron and/or carbon are calculated),
β = 51 - [% Cu] (in the case where Cu = 20 to 50%),
β = -19 + 0.4 [% Cu] (in the case where Cu = 50 to 90%).

4. An electronic or magnetic part manufactured from the alloy sheet of any one of claims 1 to 3.

5. An Fe-Cu alloy which contains, by weight, 20 to 90% Cu, 1 to 10% Cr, 0 to 10% Mo, and one or more alloying elements selected from the group consisting of Al, Sc, Y, La, Si, Ti, Zr and Hf whose amount or total amounts are not less than a calculation value of the following expression and not more than 10%, the balance, apart from impurities, being Fe: wherein α = 1,
β = 51 - [% Cu] (in the case where Cu = 20 to 50%),
β = -19 + 0.4 [% Cu] (in the case where Cu = 50 to 90%).

6. An Fe-Cu alloy which contains, by weight, 20 to 90% Cu, 1 to 10% Cr, 0 to 10% Mo, and boron and/or carbon whose amount or total amounts have a lower limit value which is a calculation value of the following expression, and have an upper limit value which is 1% when only boron is present and when both boron and carbon are present and which is 3% when only carbon is present, the balance, apart from impurities, being Fe: wherein α = 0.01,
β = 51 - [% Cu] (in the case where Cu = 20 to 50%),
β = -19 + 0.4 [% Cu] (in the case where Cu = 50 to 90%).

7. An Fe-Cu alloy which contains, by weight:
20 to 90% Cu;
1 to 10% Cr;
0 to 10% Mo;
one or more alloying elements selected from the group consisting of Al, Sc, Y, La, Si, Ti, Zr and Hf whose amount or total amounts are not less than a calculation value of the following expression and not more than 10%; and
boron and/or carbon whose amount or total amounts have a lower limit value which is a calculation value of the following expression, and have an upper limit value which is 1% when only boron is present and when both boron and carbon are present and which is 3% when only carbon is present, the balance, apart from impurities, being Fe:
wherein α = 1 (in the case where the amounts of elements belonging to the group consisting of Al, Sc, Y, La, Si, Ti, Zr and Hf are calculated),
α = 0.01 (in the case where the amounts of boron and/or carbon are calculated),
β = 51 - [% Cu] (in the case where Cu = 20 to 50%),
β = -19 + 0.4 [% Cu] (in the case where Cu = 50 to 90%).

8. The use of one or more alloying elements selected from the group consisting of Al, Sc, Y, La, Si, Ti, Zr and Hf in an amount or total amounts not less than that calculated by the following expression and not more than 10 %, in an Fe-Cu alloy comprising, by weight, 20 to 90 % Cu, 1 to 10 % Cr, 0 to 10 % Mo, the balance, apart from impurities, being iron, to reduce separation of molten forms of the alloy into iron-rich and copper-rich phases: wherein α = 1,
β = 51 - [% Cu] (in the case where Cu = 20 to 50%),
β = -19 + 0.4 [% Cu] (in the case where Cu = 50 to 90%).

9. The use of boron and/or carbon in an amount or total amounts not less than that calculated by the following expression and not more than 1 % when only boron is used or when both boron and carbon are used and not more than 3 % when only carbon is used, in an Fe-Cu alloy comprising, by weight, 20 to 90 % Cu, 1 to 10 % Cr, 0 to 10 % Mo, the balance, apart from impurities, being iron, to reduce separation of molten forms of the alloy into iron-rich and copper-rich phases: wherein α = 0.01,
β = 51 - [% Cu] (in the case where Cu = 20 to 50%),
β = -19 + 0.4 [% Cu] (in the case where Cu = 50 to 90%).

10. The use of one or more alloying elements selected from the group consisting of Al, Sc, Y, La, Si, Ti, Zr and Hf in an amount or total amounts not less than that calculated by the following expression and not more than 10 %, and boron and/or carbon in an amount or total amounts not less than that calculated by the following expression, and not more than 1 % when only boron is used and when both boron and carbon are used and not more than 3 % when only carbon is used, in an Fe-Cu alloy comprising, by weight, 20 to 90 % Cu, 1 to 10 % Cr, 0 to 10 % Mo, the balance, apart from impurities, being iron, to reduce separation of molten forms of the alloy into iron-rich and copper-rich phases: wherein α = 1, (in the case where the amounts of elements belonging to the group consisting of Al, Sc, Y, La, Si, Ti, Zr and Hf are calculated),
α = 0.01 (in the case where the amounts of boron and/or carbon are calculated),
β = 51 - [% Cu] (in the case where Cu = 20 to 50%),
β = -19 + 0.4 [% Cu] (in the case where Cu = 50 to 90%).

## Patentansprüche

1. Fe-Cu-Legierungsband, hergestellt mit einem Stranggußverfahren für dünnes Blech, wobei die Legierung, auf das Gewicht bezogen, 20 bis 90 % Cu, 1 bis 10 % Cr, 0 bis 10 % Mo und ein oder mehrere Legierungselement(e) enthält, ausgewählt aus Al, Sc, Y, La, Si, Ti, Zr und Hf, deren Menge oder Gesamtmenge nicht weniger als der aus folgendem Ausdruck berechnete Wert und nicht größer als 10 % ist, wobei der Rest, abgesehen von Verunreinigungen, Fe ist: wobei
α = 1
β = 51 - [% Cu] (im Fall, daß Cu = 20 bis 50 %),
β = -19 + 0.4 [% Cu] (im Fall, daß Cu = 50 bis 90 %).

2. Fe-Cu-Legierungsband, hergestellt mit einem Stranggußverfahren für dünnes Blech, wobei die Legierung, auf das Gewicht bezogen, 20 bis 90 % Cu, 1 bis 10 % Cr, 0 bis 10 % Mo und Bor und/oder Kohlenstoff enthält, deren Menge oder Gesamtmenge einen unteren Grenzwert aufweist, der ein aus folgendem Ausdruck berechneter Wert ist, und einen oberen Grenzwert aufweist, der 1 % ist, wenn nur Bor vorhanden ist und wenn sowohl Bor als auch Kohlenstoff vorhanden sind, und der 3 % ist, wenn nur Kohlenstoff vorhanden ist, wobei der Rest, abgesehen von Verunreinigungen, Fe ist: wobei
α = 0.01
β = 51 - [% Cu] (im Fall, daß Cu = 20 bis 50 %),
β = -19 + 0.4 [% Cu] (im Fall, daß Cu = 50 bis 90 %).

3. Fe-Cu-Legierungsband, hergestellt mit einem Stranggußverfahren für dünnes Blech, wobei die Legierung, auf das Gewicht bezogen, enthält:
20 bis 90 % Cu,
1 bis 10 % Cr,
0 bis 10 % Mo,
ein oder mehrere Legierungselement(e), ausgewählt aus Al, Sc, Y, La, Si, Ti, Zr und Hf, deren Menge oder Gesamtmenge nicht weniger als der aus folgendem Ausdruck berechnete Wert und nicht größer als 10 % ist, und
Bor und/oder Kohlenstoff, deren Menge oder Gesamtmenge einen unteren Grenzwert aufweist, der ein aus folgendem Ausdruck berechneter Wert ist, und einen oberen Grenzwert aufweist, der 1 % ist, wenn nur Bor vorhanden ist und wenn sowohl Bor als auch Kohlenstoff vorhanden sind, und der 3 % ist, wenn nur Kohlenstoff vorhanden ist, wobei der Rest, abgesehen von Verunreinigungen, Fe ist: wobei
α = 1 (im Fall, daß die Menge der Elemente, die zu der aus Al, Sc, Y, La, Si, Ti, Zr und Hf bestehenden Gruppe gehören, berechnet wird),
α = 0.01 (im Fall, daß die Menge an Bor und/oder Kohlenstoff berechnet wird).
β = 51 - [% Cu] (im Fall, daß Cu = 20 bis 50 %),
β = -19 + 0.4 [% Cu] (im Fall, daß Cu = 50 bis 90 %).

4. Elektronisches oder magnetisches Teil, hergestellt aus dem Legierungsband nach einem der Ansprüche 1 bis 3.

5. Fe-Cu-Legierung, die, auf das Gewicht bezogen, 20 bis 90 % Cu, 1 bis 10 % Cr, 0 bis 10 % Mo und ein oder mehrere Legierungselement(e) enthält, ausgewählt aus Al, Sc, Y, La, Si, Ti, Zr und Hf, deren Menge oder Gesamtmenge nicht weniger als der aus folgendem Ausdruck berechnete Wert und nicht größer als 10 % ist, wobei der Rest, abgesehen von Verunreinigungen, Fe ist: wobei
α = 1
β = 51 - [% Cu] (im Fall, daß Cu = 20 bis 50 %),
β = -19 + 0.4 [% Cu] (im Fall, daß Cu = 50 bis 90 %).

6. Fe-Cu-Legierung, die, auf das Gewicht bezogen, 20 bis 90 % Cu, 1 bis 10 % Cr, 0 bis 10 % Mo und Bor und/oder Kohlenstoff enthält, deren Menge oder Gesamtmenge einen unteren Grenzwert aufweist, der ein aus folgendem Ausdruck berechneter Wert ist, und einen oberen Grenzwert aufweist, der 1 % ist, wenn nur Bor vorhanden ist und wenn sowohl Bor als auch Kohlenstoff vorhanden sind, und der 3 % ist, wenn nur Kohlenstoff vorhanden ist, wobei der Rest, abgesehen von Verunreinigungen, Fe ist: wobei
α = 0.01
β = 51 - [% Cu] (im Fall, daß Cu = 20 bis 50 %),
β = -19 + 0.4 [% Cu] (im Fall, daß Cu = 50 bis 90 %).

7. Fe-Cu-Legierung, die, auf das Gewicht bezogen,
20 bis 90 % Cu,
1 bis 10 % Cr,
0 bis 10 % Mo,
ein oder mehrere Legierungselement(e), ausgewählt aus Al, Sc, Y, La, Si, Ti, Zr und Hf, deren Menge oder Gesamtmenge nicht weniger als der aus folgendem Ausdruck berechnete Wert und nicht größer als 10 % ist, und
Bor und/oder Kohlenstoff enthält, deren Menge oder Gesamtmenge einen unteren Grenzwert aufweist, der ein aus folgendem Ausdruck berechneter Wert ist, und einen oberen Grenzwert aufweist, der 1 % ist, wenn nur Bor vorhanden ist und wenn sowohl Bor als auch Kohlenstoff vorhanden sind, und der 3 % ist, wenn nur Kohlenstoff vorhanden ist, wobei der Rest, abgesehen von Verunreinigungen, Fe ist: wobei
α = 1 (im Fall, daß die Menge der Elemente, die zu der aus Al, Sc, Y, La, Si, Ti, Zr und Hf bestehenden Gruppe gehören, berechnet wird),
α = 0.01 (im Fall, daß die Menge an Bor und/oder Kohlenstoff berechnet wird).
β = 51 - [% Cu] (im Fall, daß Cu = 20 bis 50 %),
β = -19 + 0.4 [% Cu] (im Fall, daß Cu = 50 bis 90 %).

8. Verwendung eines oder mehrerer Legierungselemente, ausgewählt aus Al, Sc, Y, La, Si, Ti, Zr und Hf in einer nicht geringeren Menge oder Gesamtmenge als die aus folgendem Ausdruck berechnete und nicht mehr als 10 %, in einer Fe-Cu-Legierung, umfassend, auf das Gewicht bezogen, 20 bis 90 % Cu, 1 bis 10 % Cr, 0 bis 10 % Mo, wobei der Rest, abgesehen von Verunreinigungen, Eisen ist, um die Auftrennung von geschmolzenen Formen der Legierung in eisenreiche und kupferreiche Phasen zu vermindern: wobei
α = 1
β = 51 - [% Cu] (im Fall, daß Cu = 20 bis 50 %),
β = -19 + 0.4 [% Cu] (im Fall, daß Cu = 50 bis 90 %).

9. Verwendung von Bor und/oder Kohlenstoff in einer nicht geringeren Menge oder Gesamtmenge als die aus folgendem Ausdruck berechnete und nicht mehr als 1 %, wenn nur Bor verwendet wird oder wenn sowohl Bor als auch Kohlenstoff verwendet werden, und nicht mehr als 3 %, wenn nur Kohlenstoff verwendet wird, in einer Fe-Cu-Legierung, umfassend, auf das Gewicht bezogen, 20 bis 90 % Cu, 1 bis 10 % Cr, 0 bis 10 % Mo, wobei der Rest, abgesehen von Verunreinigungen, Eisen ist, um die Auftrennung von geschmolzenen Formen der Legierung in eisenreiche und kupferreiche Phasen zu vermindern: wobei
α = 0.01
β = 51 - [% Cu] (im Fall, daß Cu = 20 bis 50 %),
β = -19 + 0.4 [% Cu] (im Fall, daß Cu = 50 bis 90 %).

10. Verwendung eines oder mehrerer Legierungselemente, ausgewählt aus Al, Sc, Y, La, Si, Ti, Zr und Hf in einer nicht geringeren Menge oder Gesamtmenge als die aus folgendem Ausdruck berechnete und nicht mehr als 10 %, und Bor und/oder Kohlenstoff in einer nicht geringeren Menge oder Gesamtmenge als die aus folgendem Ausdruck berechnete und nicht mehr als 1 %, wenn nur Bor verwendet wird und wenn sowohl Bor als auch Kohlenstoff verwendet werden, und nicht mehr als 3 %, wenn nur Kohlenstoff verwendet wird, in einer Fe-Cu-Le-gierung, umfassend, auf das Gewicht bezogen, 20 bis 90 % Cu, 1 bis 10 % Cr, 0 bis 10 % Mo, wobei der Rest, abgesehen von Verunreinigungen, Eisen ist, um die Auftrennung von geschmolzenen Formen der Legierung in eisenreiche und kupferreiche Phasen zu vermindern: wobei
α = 1 (im Fall, daß die Menge der Elemente, die zu der aus Al, Sc, Y, La, Si, Ti, Zr und Hf bestehenden Gruppe gehören, berechnet wird),
α = 0.01 (im Fall, daß die Menge an Bor und/oder Kohlenstoff berechnet wird).
β = 51 - [% Cu] (im Fall, daß Cu = 20 bis 50 %),
β = -19 + 0.4 [% Cu] (im Fall, daß Cu = 50 bis 90 %).

## Revendications

1. Feuille en alliage Fe-Cu, fabriquée par un procédé de coulage continu en plaque mince, l'alliage contenant, en poids, 20 à 90 % de Cu, 1 à 10 % de Cr, 0 à 10 % de Mo, et un ou plusieurs éléments d'alliage choisis dans le groupe constitué de Aℓ, Sc, Y, La, Si, Ti, Zr et Hf, dont la quantité ou les quantités totales ne sont pas inférieures à une valeur de calcul de l'expression suivante et pas supérieures à 10 %, le reste, à part les impuretés, étant Fe : où
α = 1,
β = 51 - [% de Cu] (dans le cas où Cu = 20 à 50 %),
β = -19 + 0,4 [% de Cu] (dans le cas où Cu = 50 à 90 %).

2. Feuille en alliage Fe-Cu fabriquée par un procédé de coulage continu en plaque mince, l'alliage contenant, en poids, 20 à 90 % de Cu, 1 à 10 % de Cr, 0 à 10 % de Mo, et du bore et/ou du carbone, dont la quantité ou les quantités totales ont une valeur limite inférieure qui est une valeur de calcul de l'expression suivante, et ont une valeur limite supérieure qui est 1 % lorsque seul -le bore est présent et lorsque tant le bore que le carbone sont présents, et qui est 3 % lorsque seul le carbone est présent, le reste, à part les impuretés, étant Fe : où
α = 0,01,
β = 51 - [% de Cu] (dans le cas où Cu = 20 à 50 %),
β = -19 + 0,4 [% de Cu] (dans le cas où Cu = 50 à 90 %).

3. Feuille en alliage Fe-Cu fabriquée par un procédé de coulage continu en plaque mince, l'alliage contenant, en poids :
20 à 90 % de Cu ;
1 à 10 % de Cr ;
0 à 10 % de Mo ;
un ou plusieurs éléments d'alliage choisis dans le groupe constitué de Aℓ, Sc, Y, La, Si, Ti, Zr et Hf, dont la quantité ou les quantités totales ne sont pas inférieures à une valeur de calcul de l'expression suivante et pas supérieures à 10 % ; et
du bore et/ou du carbone, dont la quantité ou les quantités totales ont une valeur limite inférieure qui est une valeur de calcul de l'expression suivante, et ont une valeur limite supérieure qui est 1 % lorsque seul le bore est présent et lorsque tant le bore que le carbone sont présents, et qui est 3 % lorsque seul le carbone est présent, le reste, à part les impuretés, étant Fe : où
α = 1 (dans le cas où les quantités d'éléments appartenant au groupe constitué de Aℓ, Sc, Y, La, Si, Ti, Zr et Hf sont calculées),
α = 0,01 (dans le cas où les quantités de bore et/ou de carbone sont calculées),
β = 51 - [% de Cu] (dans le cas où Cu = 20 à 50 %),
β = -19 + 0,4 [% de Cu] (dans le cas où Cu = 50 à 90 %).

4. Pièce électronique ou magnétique fabriquée à partir de la feuille en alliage selon l'une quelconque des revendications 1 à 3.

5. Alliage Fe-Cu qui contient, en poids, 20 à 90 % de Cu, 1 à 10 % de Cr, 0 à 10 % de Mo, et un ou plusieurs éléments d'alliage choisis dans le groupe constitué de Aℓ, Sc, Y, La, Si, Ti, Zr et Hf, dont la quantité ou les quantités totales ne sont pas inférieures à une valeur de calcul de l'expression suivante et pas supérieures à 10 %, le reste, à part les impuretés, étant Fe : où
α = 1,
β = 51 - [% de Cu] (dans le cas où Cu = 20 à 50 %),
β = -19 + 0,4 [% de Cu] (dans le cas où Cu = 50 à 90 %).

6. Alliage Fe-Cu qui contient, en poids, 20 à 90 % de Cu, 1 à 10 % de Cr, 0 à 10 % de Mo, et du bore et/ou du carbone, dont la quantité ou les quantités totales ont une valeur limite inférieure qui est une valeur de calcul de l'expression suivante, et ont une valeur limite supérieure qui est 1 % lorsque seul le bore est présent et lorsque tant le bore que le carbone sont présents, et qui est 3 % lorsque seul le carbone est présent, le reste, à part les impuretés, étant Fe : où
α = 0,01,
β = 51 - [% de Cu] (dans le cas où Cu = 20 à 50 %),
β = -19 + 0,4 [% de Cu] (dans le cas où Cu = 50 à 90 %).

7. Alliage Fe-Cu qui contient, en poids :
20 à 90 % de Cu ;
1 à 10 % de Cr ;
0 à 10 % de Mo ;
un ou plusieurs éléments d'alliage choisis dans le groupe constitué de Aℓ, Sc, Y, La, Si, Ti, Zr et Hf, dont la quantité ou les quantités totales ne sont pas inférieures à une valeur de calcul de l'expression suivante et pas supérieures à 10 % ; et
du bore et/ou du carbone, dont la quantité ou les quantités totales ont une valeur limite inférieure qui est une valeur de calcul de l'expression suivante, et ont une valeur limite supérieure qui est 1 % lorsque seul le bore est présent et lorsque tant le bore que le carbone sont présents, et qui est 3 % lorsque seul le carbone est présent, le reste, à part les impuretés, étant Fe : où
α = 1 (dans le cas où les quantités d'éléments appartenant au groupe constitué de Aℓ, Sc, Y, La, Si, Ti, Zr et Hf sont calculées),
α = 0,01 (dans le cas où les quantités de bore et/ou de carbone sont calculées),
β = 51 - [% de Cu] (dans le cas où Cu = 20 à 50 %),
β = -19 + 0,4 [% de Cu] (dans le cas où Cu = 50 à 90 %).

8. Utilisation d'un ou plusieurs éléments d'alliage choisis dans le groupe constitué de Aℓ, Sc, Y, La, Si, Ti, Zr et Hf, en une quantité ou en quantités totales non inférieures à celle calculée par l'expression suivante et non supérieures à 10 %, dans un alliage Fe-Cu comprenant, en poids, 20 à 90 % de Cu, 1 à 10 % de Cr, 0 à 10 % de Mo, le reste, à part les impuretés, étant du fer, pour réduire la séparation des formes fondues de l'alliage en phases riches en fer et riches en cuivre : où
α = 1,
β = 51 - [% de Cu] (dans le cas où Cu = 20 à 50 %),
β = -19 + 0,4 [% de Cu] (dans le cas où Cu = 50 à 90 %).

9. Utilisation de bore et/ou de carbone, en une quantité ou en quantités totales non inférieures à celle calculée par l'expression suivante et non supérieures à 1 % lorsque seul le bore est utilisé ou lorsque tant le bore que le carbone sont utilisés, et non supérieures à 3 % lorsque seul le carbone est utilisé, dans un alliage Fe-Cu comprenant, en poids, 20 à 90 % de Cu, 1 à 10 % de Cr, 0 à 10 % de Mo, le reste, à part les impuretés, étant du fer, pour réduire la séparation des formes fondues de l'alliage en phases riches en fer et riches en cuivre : où
α = 0,01,
β = 51 - [% de Cu] (dans le cas où Cu = 20 à 50 %),
β = -19 + 0,4 [% de Cu] (dans le cas où Cu = 50 à 90 %).

10. Utilisation d'un ou plusieurs éléments d'alliage choisis dans le groupe constitué de Aℓ, Sc, Y, La, Si, Ti, Zr et Hf, en une quantité ou en quantités totales non inférieures à celle calculée par l'expression suivante et non supérieures à 10 %, et de bore et/ou de carbone en une quantité ou en quantités totales non inférieures à celle calculée par l'expression suivante, et non supérieures à 1 % lorsque seul le bore est utilisé ou lorsque tant le bore que le carbone sont utilisés, et non supérieures à 3 % lorsque seul le carbone est utilisé, dans un alliage Fe-Cu comprenant, en poids, 20 à 90 % de Cu, 1 à 10 % de Cr, 0 à 10 % de Mo, le reste, à part les impuretés, étant du fer, pour réduire la séparation des formes fondues de l'alliage en phases riches en fer et riches en cuivre ; où
α = 1 (dans le cas où les quantités d'éléments appartenant au groupe constitué de Aℓ, Sc, Y, La, Si, Ti, Zr et Hf sont calculées),
α = 0,01 (dans le cas où les quantités de bore et/ou de carbone sont calculées),
β = 51 - [% de Cu] (dans le cas où Cu = 20 à 50 %),
β = -19 + 0,4 [% de Cu] (dans le cas où Cu = 50 à 90 %).
